

## UNITED STATES PATENT OFFICE

ARTHUR S. ROBERTS, OF HENDERSONVILLE, NORTH CAROLINA

## METHOD OF CROSS-DYEING FABRICS

No Drawing. Application filed December 17, 1927, Serial No. 240,919. Renewed December 11, 1930.

My invention relates to a process of dyeing cotton and that type of regenerated cellulose known as xanthate silk, or viscose, when woven in the same fabric.

5 An object of my invention is to provide a combination of certain dyestuffs and chemicals which will act to dye either the cotton or a type of regenerated cellulose and leave the other portion of the fabric undyed.

10 Another object of my invention is to provide a process of dyeing fabrics woven from cotton and certain types of regenerated cellulose in which the cotton may be dyed one color and the regenerated cellulose dyed 15 another color.

It has heretofore been claimed by those skilled in the art of dyeing fabrics that a fabric composed of cotton and xanthate silk or viscose cannot be dyed in any manner 20 other than that of dyeing both the cotton and the xanthate silk or viscose of the same color, due to the fact that cotton and viscose have practically the same affinity for all 25 dyes.

25 It is the purpose of this invention to set forth a method and means whereby cotton and viscose, or xanthate silk, can be made to accept certain and distinct colors when woven, spun or knitted into the same fabric by 30 a certain careful selection of dyes for the purpose and by regulating the temperatures of the dye baths as well as regulating the amount of chemicals added to the dye bath, and by dyeing each fiber in a separate dye 35 bath, or in some cases, by combining the two dyebaths and dyeing two separate and distinct colors at one and the same operation, the art of which is known as "cross-dyeing". I am aware that the art of cross- 40 dyeing has been used heretofore for various textiles woven of different materials, but, as stated, there has not heretofore been used any method whereby cotton and regenerated cellulose of the viscose type, when woven 45 in the same fabric can be dyed separate and distinct colors either by separate dyeing or by one operation.

I have discovered by using certain families of neutral dyeing acid wool dyes, such 50 as wool yellow ex. Schultz Number 23, wool

blue R. Schultz Number 188, new red 5R, Schultz Number 168 and the like which will when combined with glycerine, or acidified boil off oil to act as a penetrant, will when introduced into a dye machine containing sufficient water at a temperature, of approximately 180 degrees Fahrenheit together with or without the addition of sodium sulphate or Glauber's salt form a dyebath that will 55 dye the viscose or xanthate silk to the color and shade desired, and leave the cotton undyed or only slightly stained. It is, of course, to be understood that one or more of the dyes such as wool yellow extra, wool blue R, or new red 5R may be used at a time, 60 as in some cases only one of these dyes would be desired, while a combination of two or more of neutral dyeing acid dyes might be desired to produce the proper 65 color.

I have also discovered that certain selected substantive or direct dyes, selected from the group consisting of direct yellow S 2 G, Schultz, No. 10—direct rubine B, Schultz No. 313—direct brilliant blue G, Schultz No. 415 and the like, together or without the addition of sulphonated oil, will when introduced into a dye machine containing sufficient water at a temperature of approximately 120 degrees F. form a dyebath that 70 will act to dye the cotton to a shade desired and leave the xanthate silk or viscose undyed or only slightly stained. It is, of course, to be understood that I may use all 75 the above named substantive or direct dyes at one time or may use one or more of the same according to the shade desired to be produced, although I do not desire to be bound by the explanation which follows.

I have found that the best process for the cross-dyeing of cotton and viscose or xanthate silk with the dyes above named is substantially as follows for best results: One or more of the neutral acid dyes for dyeing the viscose of the neutral acid group is first pasted down with glycerine or slightly acidified boil off oil, then dissolved in boiling water and strained into the dye machine with the necessary amount of water for the work, which has been heated to ap- 80 85 90 95 100

proximately 180 degrees Fahrenheit. The cloth which has been previously wet out in cold water is then run into the machine and given from three to five dips or ends in this 5 dyebath in order to obtain the shade desired. This bath is then wasted and the cloth given a slight rinse in cold water in order to clear the dyes from the cotton part of the fabric.

The dyebath composed of one or more of 10 the substantive or direct dyes may then be dissolved and poured into the machine containing sufficient water at a temperature of approximately 120 degrees Fahrenheit and the goods are likewise given from three to 15 five dips or ends in this dye liquor in order to bring up the shade desired on the cotton part of the fabric. This liquor is again wasted and the goods given a good rinsing in cold water after which the goods are 20 squeezed and dried.

In the case of a combined dyebath, I have found that by making up a dyebath composed of the necessary amount of the wool yellow extra, the acidified boil off oil, the direct rubine B. conc. together with sufficient water at a temperature of approximately 180 degrees Fahrenheit and giving the cloth containing the viscose or xanthate silk and cotton fibres from three to five ends or dips 25 necessary to produce the shade desired, a very beautiful red and gold combination can be produced in one bath at one and the same operation. The last paragraph merely gives an explanation of the results produced by 30 securing two dyes according to my process and I desire it to be understood that any combination of the dyes enumerated in this application may be used when it is desired to produce a certain shade in either the viscose 35 or the cotton fibres.

In the specification, I have set forth a preferred embodiment of my invention, and although specific terms are employed, they are used in a generic and descriptive sense 45 only and not for purposes of limitation, the scope of my invention being set forth in the appended claims.

I claim:

1. That method of dyeing a fabric composed of viscose and cotton which comprises wetting the fabric with water, subjecting the fabric to a dyebath containing neutral dyeing acid dyes selected from the group consisting of wool yellow extra, Schultz Number 23, wool blue R, Schultz Number 188, and new red 5R, Schultz Number 248, and glycerine, rinsing the fabric in water, then subjecting the fabric to a dyebath containing substantive dyes selected from the group 50 consisting of direct yellow S 2 G, Schultz Number 10, direct rubine B concentrated, Schultz Number 313, and direct blue 6 G extra, Schultz Number 415 and sulphonated oil, and then rinsing the dyed fabric in 55 water.

2. That method of dyeing a fabric containing viscose and cotton fibres which comprises subjecting the fabric successively to dyebaths containing neutral dyeing acid dyes selected from the group consisting of wool yellow extra, Schultz Number 23, wool blue R, Schultz Number 188, and new red 5R, Schultz Number 248, and to a bath containing substantive direct dyes selected from the group consisting of direct yellow S 2 G, Schultz Number 10, direct rubine B concentrated, Schultz Number 313, and direct blue 6 G extra, Schultz Number 415. 70

3. That method of cross-dyeing a fabric containing viscose and cotton fibres which comprises subjecting the fabric to a dyebath containing neutral dyeing acid dyes selected from the group consisting of wool yellow extra, Schultz Number 23, wool blue R, Schultz Number 188, and new red 5R, Schultz Number 248, heated to a temperature of approximately 180 degrees Fahrenheit, and then subjecting the fabric to a substantive direct dyebath selected from the group consisting of direct yellow S 2 G, Schultz Number 10, direct rubine B concentrated, Schultz Number 313, and direct blue 6 G extra, Schultz Number 415 heated to a temperature of approximately 120 degrees Fahrenheit. 80

4. That method of cross-dyeing a fabric containing viscose and cotton fibres which comprises subjecting the fabric to a dyebath containing neutral acid dyes selected from the group consisting of wool yellow extra, Schultz Number 23, wool blue R, Schultz Number 188, and new red 5R, Schultz Number 248 to dye the viscose and then subjecting the fabric to a dyebath containing substantive direct dyes selected from the group consisting of direct yellow S 2 G, Schultz Number 10, direct rubine B concentrated, Schultz Number 313, and direct blue 6 G extra, Schultz Number 415 to dye the cotton fibres. 90

5. That method of dyeing a fabric composed of viscose and cotton to impart one color to the viscose and another color to the cotton which comprises subjecting the fabric to a dyebath containing neutral dyeing acid dyes selected from the group consisting of wool yellow extra, Schultz Number 23, wool blue R, Schultz Number 188, and new red 5R, Schultz Number 248; to dye the viscose fibres and then subjecting the fabric to a dyebath containing substantive direct dyes selected from the group consisting of direct yellow S 2 G, Schultz Number 10, direct rubine B concentrated, Schultz Number 313, and direct blue 6 G extra, Schultz Number 415 to dye the cotton another color. 100

6. That method of dyeing a fabric composed of viscose and cotton fibres to impart different colors to the two sets of fibres which comprises subjecting the fabric to a 105

- dyebath containing neutral dyeing acid dyes selected from the group consisting of wool yellow extra, Schultz Number 23, wool blue R, Schultz Number 188, and new red 5R, Schultz Number 248 and then subjecting the fabric to a dyebath containing substantive dyes selected from the group consisting of direct yellow S 2 G, Schultz Number 10, direct rubine B concentrated, Schultz Number 313, and direct blue 6 G extra, Schultz Number 415 and acidified boil off oil, whereby the viscose fibres are dyed one color and the cotton fibres are dyed another color.
7. That method of dyeing a fabric composed of regenerated cellulose and cotton fibres to impart different colors to the two sets of fibres which comprises subjecting the fabric to a dyebath containing neutral dyeing acid dyes selected from the group consisting of wool yellow extra, Schultz Number 23, wool blue R, Schultz Number 188, and new red 5R, Schultz Number 248 and then subjecting the fabric to a dyebath containing substantive dyes selected from the group consisting of direct yellow S 2 G, Schultz Number 10, direct rubine B concentrated, Schultz Number 313, and direct blue 6 G extra, Schultz Number 415 and acidified boil off oil, whereby the regenerated cellulose fibres are dyed one color and the cotton fibres are dyed another color.
8. That method of dyeing a fabric comprising viscose and cotton fibres, which comprises subjecting the fabric to a dyebath containing neutral dyeing acid dyes selected from the group consisting of wool yellow extra, Schultz Number 23, wool blue R, Schultz Number 188, and new red 5R, Schultz Number 248 to dye the viscose fibres and to leave the cotton fibres substantially undyed.

In testimony whereof I affix my signature.  
ARTHUR S. ROBERTS.

45

50

55

60

65